



US010086237B1

(12) **United States Patent**  
**Chavan et al.**

(10) **Patent No.:** **US 10,086,237 B1**  
(45) **Date of Patent:** **Oct. 2, 2018**

(54) **GRAPHENE AND CARBON NANOTUBE REINFORCED GOLF BALL**

(71) Applicant: **Callaway Golf Company**, Carlsbad, CA (US)

(72) Inventors: **Vijay Chavan**, Vista, CA (US); **David Bartels**, Carlsbad, CA (US)

(73) Assignee: **Callaway Golf Company**, Carlsbad, CA (US)

(\*) Notice: Subject to any disclaimer, the term of this patent is extended or adjusted under 35 U.S.C. 154(b) by 0 days.

(21) Appl. No.: **15/729,231**

(22) Filed: **Oct. 10, 2017**

**Related U.S. Application Data**

(63) Continuation-in-part of application No. 15/436,169, filed on Feb. 17, 2017, now Pat. No. 9,789,366.

(60) Provisional application No. 62/401,034, filed on Sep. 28, 2016.

(51) **Int. Cl.**

**A63B 37/06** (2006.01)

**A63B 37/00** (2006.01)

(52) **U.S. Cl.**

CPC ..... **A63B 37/0039** (2013.01); **A63B 37/005** (2013.01); **A63B 37/0023** (2013.01); **A63B 37/0075** (2013.01); **A63B 37/0076** (2013.01)

(58) **Field of Classification Search**

CPC ..... A63B 37/005; A63B 37/0076; A63B 37/0051

USPC ..... 473/376

See application file for complete search history.

(56)

**References Cited**

**U.S. PATENT DOCUMENTS**

|             |          |                             |
|-------------|----------|-----------------------------|
| 1,191,383 A | 7/1916   | Aylsworth                   |
| 3,492,197 A | 1/1970   | Olstowski et al.            |
| 4,844,471 A | 7/1989   | Terence et al.              |
| 4,911,451 A | 3/1990   | Sullivan et al.             |
| 4,986,545 A | 1/1991   | Sullivan                    |
| 5,048,838 A | 9/1991   | Chikaraishi et al.          |
| 5,252,652 A | 10/1993  | Egashira et al.             |
| 5,588,924 A | 12/1996  | Sullivan et al.             |
| 5,688,595 A | 11/1997  | Yamagishi et al.            |
| 5,721,304 A | 2/1998   | Pasqua                      |
| 5,725,442 A | 3/1998   | Higuchi et al.              |
| 5,779,562 A | 7/1998   | Melvin et al.               |
| 5,816,937 A | 10/1998  | Shimosaka et al.            |
| 5,830,086 A | 11/1998  | Hayashi et al.              |
| 5,980,396 A | 11/1999  | Moriyama et al.             |
| 6,117,025 A | * 9/2000 | Sullivan ..... A63B 37/0003 |

473/373

|              |         |                 |
|--------------|---------|-----------------|
| 6,117,026 A  | 9/2000  | Hayashi et al.  |
| 6,123,630 A  | 9/2000  | Hayashi et al.  |
| 6,142,886 A  | 11/2000 | Sullivan et al. |
| 6,248,027 B1 | 6/2001  | Hayashi et al.  |
| 6,251,031 B1 | 6/2001  | Hayashi et al.  |
| 6,277,034 B1 | 8/2001  | Nesbitt et al.  |
| 6,299,550 B1 | 10/2001 | Molitor et al.  |
| 6,361,454 B1 | 3/2002  | Yoshida et al.  |
| 6,443,858 B2 | 9/2002  | Bartels et al.  |

(Continued)

*Primary Examiner* — Raeann Gorden

(74) *Attorney, Agent, or Firm* — Michael A. Catania; Sonia Lari; Rebecca Hanovice

(57) **ABSTRACT**

A golf ball comprising an inner core comprising polybutadiene, and an outer core comprising a polybutadiene material, a graphene material and a carbon nanotube material (CNT) is disclosed herein. Improved durability of the core by using a mixture of graphene and CNT can result in higher mean time to fail (MTTF) upon repeated impact in a high speed testing device, or with a golf club in normal play.

**14 Claims, 14 Drawing Sheets**



| (56)                  | References Cited |         |                    |              |      |
|-----------------------|------------------|---------|--------------------|--------------|------|
| U.S. PATENT DOCUMENTS |                  |         |                    |              |      |
| 6,461,251             | B1               | 10/2002 | Yamagishi et al.   | 7,918,748    | B2   |
| 6,461,253             | B2               | 10/2002 | Ogg                | 8,025,593    | B2   |
| 6,468,169             | B1               | 10/2002 | Hayashi et al.     | 8,109,843    | B2   |
| 6,478,697             | B2               | 11/2002 | Yagley et al.      | 8,425,351    | B2   |
| 6,482,345             | B1               | 11/2002 | Dewanjee           | 8,475,298    | B2   |
| 6,495,633             | B1               | 12/2002 | Sullivan et al.    | 8,651,976    | B1   |
| 6,520,870             | B2               | 2/2003  | Tzivanis et al.    | 8,876,635    | B1   |
| 6,565,455             | B2               | 5/2003  | Hayashi et al.     | 8,974,318    | B1 * |
| 6,565,456             | B2               | 5/2003  | Hayashi et al.     | 9,370,694    | B2   |
| 6,626,770             | B2               | 9/2003  | Takemura et al.    | 9,393,462    | B2   |
| 6,653,382             | B1               | 11/2003 | Statz et al.       | 2002/0065149 | A1   |
| 6,685,579             | B2               | 2/2004  | Sullivan           | 2002/0165045 | A1   |
| 6,705,956             | B1               | 3/2004  | Moriyama et al.    | 2005/0020385 | A1   |
| 6,743,122             | B2               | 6/2004  | Hayashi et al.     | 2005/0037866 | A1   |
| 6,849,006             | B2               | 2/2005  | Cavallaro et al.   | 2005/0250601 | A1   |
| 6,994,638             | B2               | 2/2006  | Rajagopalan et al. | 2005/0272867 | A1   |
| 7,121,959             | B1               | 10/2006 | Yoshida et al.     | 2006/0264269 | A1   |
| 7,220,191             | B2               | 5/2007  | Onoda et al.       | 2006/0270790 | A1   |
| 7,226,367             | B2               | 6/2007  | Higuchi et al.     | 2008/0058121 | A1   |
| 7,303,490             | B2               | 12/2007 | Takesue et al.     | 2013/0165261 | A1   |
| 7,335,114             | B2               | 2/2008  | Hebert et al.      | 2015/0133593 | A1   |
| 7,361,102             | B2               | 4/2008  | Ladd et al.        | 2015/0343270 | A1   |
| 7,537,531             | B2               | 5/2009  | Ladd et al.        | 2015/0375051 | A1   |
| 7,591,741             | B2               | 9/2009  | Sullivan et al.    | 2015/0375062 | A1   |
| 7,874,939             | B2               | 1/2011  | Sullivan et al.    | 2016/0279482 | A1 * |

\* cited by examiner

473/376

A63B 37/0076

473/376



FIG. 1



FIG. 2



FIG. 3



FIG. 4



FIG. 5



FIG. 5A



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19

**FIG. 20**

**GRAPHENE AND CARBON NANOTUBE  
REINFORCED GOLF BALL**

**CROSS REFERENCES TO RELATED  
APPLICATIONS**

The Present Application is a continuation-in-part application of U.S. patent application Ser. No. 15/436,169, filed on Feb. 17, 2017, which claims priority to U.S. Provisional Patent Application No. 62/401,034, filed on Sep. 28, 2016, each of which is hereby incorporated by reference in its entirety.

**STATEMENT REGARDING FEDERALLY  
SPONSORED RESEARCH OR DEVELOPMENT**

Not Applicable

**BACKGROUND OF THE INVENTION**

**Field of the Invention**

The present invention generally relates to the use of graphene and carbon nanotubes in layers of a golf ball.

**Description of the Related Art**

Graphene based nanocomposites perform the best when there is a good separation between layers of graphene nanoplatelets. Since nanoplatelets have a strong tendency to stick to each other, observed improvement in physical properties is lower than theoretically expected. Various techniques to prevent stacking or agglomeration of graphene nanoplatelets can be found in literature. These methods include chemical modification such as grafting or addition of other nanofillers that occupy spaces between layers of graphene. Later approach is more important since it is more convenient than chemical modification. One such nanofillers is carbon nanotubes, which as the name suggests is tubular in nature. When graphene and CNT are mixed together, one-dimensional CNTs occupy spaces between layers of graphene. This improves quality of graphene dispersion in a given polymer matrix.

The prior art observed significant improvement in high specific capacitance by replacing 10% graphene with CNT. Other references mention use of one dimensional CNT in a graphene based epoxy composite that shows much better mechanical properties than epoxy composite that uses either graphene or CNT. They explain de-aggregation of graphene with what looks like a paper and pencil model. Graphene which is two dimensional is prevented from stacking due to presence of pencil like carbon nanotubes. Authors observed higher tensile strength, elongation, as well as higher thermal conductivity for epoxy composites that used a mixture of graphene and CNT compared to epoxy composites that used only either of the two. Other references used a mixture of three allotropes of carbon: graphene, CNT, and carbon black to achieve a very high electrical conductivity in an epoxy composite. Conductivity of composite with all these three fillers was shown to be higher than the conductivity of a composite that used either one or two of these allotropes. Authors attributed this remarkable increase in electrical conductivity to de-aggregation of graphene layers by CNT and carbon black. Other references discuss use of CNT in a graphene polyaniline (PANT) composite for super-capacitor application. They describe CNT as tiny nanosized wires that further improve conductivity of graphene/PANI composite

by interconnecting layers of graphene. Authors describe this hybrid composite similar to paper/pencil model where layers of graphene/PANI are inter connected by nanowires of CNT. Other references describe mixing graphene oxide and oxidized CNT solution together and later reducing the mixture to obtain reduced graphene/CNT composite. These authors show presence of CNT stashed between layers of graphene that causes increase in electrical conductivity of final composite. Other references use a mixture of CNT and graphene in polypropylene (PP) matrix. Other references observed 2-7-fold reduction in electrical resistance upon incorporation of CNT to a graphene PP composite. This increased conductivity was attributed to CNTs bridging layers of graphene sheets.

There exists a need to design a stronger golf ball core that utilizes both graphene and carbon nanotube. This proposed mixture of two nanofillers will improve the spacing between graphene nanoplatelets resulting in improved mechanical strength and thermal conductivity of core composite material. Increased mechanical strength results in golf ball core that lasts longer. Increased thermal conductivity results in more uniform/faster curing of core that can reduce cure time and increase throughput.

**BRIEF SUMMARY OF THE INVENTION**

The primary purpose of the present invention is to improve durability of golf ball core by incorporation of mixture of graphene and CNT in the core to improve the impact strength of the ball. This benefit can be seen in either a ball with single piece core, or a dual core with an outer core firmer than the inner core. Improved durability of the core by using a mixture of graphene and CNT can result in higher mean time to fail (MTTF) upon repeated impact in a high speed testing device, or with a golf club in normal play.

Another objective is to improve aging properties due to the incorporation of graphene in the core for better retention of compression and COR over time.

One aspect of the present invention is a golf ball comprising an inner core comprising polybutadiene, an outer core comprising a polybutadiene material, a graphene material in an amount ranging from 0.01 to 6.0 weight percent of the outer core, and a carbon nanotube material (CNT) in an amount ranging from 0.01 to 6.0 weight percent of the outer core, and a cover layer.

In a more preferred embodiment, the graphene material ranges from 0.4 to 1.0 weight percent of the outer core. In an even more preferred embodiment, the graphene material ranges from 0.4 to 0.8 weight percent of the outer core.

Durability of the dual core with a high compression differential is greatly enhanced by incorporation of graphene and CNT mixture in outer core. The graphene and CNT reinforcement to the outer core helps resist the high stresses experienced by the core when struck at high club speeds.

Graphene/CNT can be added in powder or a masterbatch form. Masterbatch with polybutadiene or polyisoprene as a carrier can further improve dispersion of graphene/CNT in core mixture.

Due to high thermal conductivity of graphene/CNT, overall thermal conductivity of cores can be improved. With higher thermal conductivity, curing cycles can be made shorter. Shorter curing cycles can lead to higher output in production.

Optionally, carbon black can be added to this mixture to make a core based on three nanofillers: Graphene, CNT, and carbon black.

Another aspect of the present invention is a golf ball comprising an inner core, an outer core, an inner mantle layer, an outer mantle layer, and a cover. The outer core comprises a polybutadiene material, a graphene material in an amount ranging from 0.01 to 6.0 weight percent of the outer core, and a carbon nanotube material (CNT) in an amount ranging from 0.01 to 6.0 weight percent of the outer core. The outer core is disposed over the inner core. The inner mantle layer is disposed over the outer core. The inner mantle layer has a thickness ranging from 0.03 inch to 0.09 inch. The inner mantle layer is composed of an ionomer material. The inner mantle layer material has a plaque Shore D hardness ranging from 34 to 55. The outer mantle layer is disposed over the inner mantle layer. The outer mantle layer has a thickness ranging from 0.025 inch to 0.050 inch. The cover layer is disposed over the outer mantle layer. The cover layer has a thickness ranging from 0.025 inch to 0.040 inch. The cover layer has a lower Shore D hardness than the outer mantle layer. The outer mantle layer has a higher Shore D hardness than the inner mantle layer. The outer core has a higher Shore D hardness than the inner mantle layer and the center core.

Yet another aspect of the present invention is a golf ball comprising an inner core, an outer core, an inner mantle layer, an outer mantle layer, and a cover. The outer core comprises a polybutadiene material, a graphene material in an amount ranging from 0.01 to 6.0 weight percent of the outer core, and a carbon nanotube material (CNT) in an amount ranging from 0.01 to 6.0 weight percent of the outer core. The outer core is disposed over the inner core. The inner mantle layer is disposed over the outer core. The inner mantle layer has a thickness ranging from 0.03 inch to 0.09 inch. The inner mantle layer material has a plaque Shore D hardness ranging from 30 to 50. The outer mantle layer is disposed over the inner mantle layer. The outer mantle layer has a thickness ranging from 0.025 inch to 0.070 inch. The outer mantle layer material has a plaque Shore D hardness ranging from 50 to 71. The inner mantle is thicker than the outer mantle, and the outer mantle is harder than the inner mantle. The cover layer is disposed over the outer mantle layer. The cover layer has a thickness ranging from 0.025 inch to 0.050 inch. The cover layer has a Shore D hardness less than the hardness of the outer mantle layer. The outer mantle layer has a higher Shore D hardness than the inner mantle layer. The outer core has a higher Shore D hardness than the inner mantle layer and the center core.

Yet another aspect of the present invention is a golf ball comprising an inner core, an outer core, an inner mantle layer, an outer mantle layer, and a cover. The outer core comprises a polybutadiene material, a graphene material in an amount ranging from 0.01 to 6.0 weight percent of the outer core, and a carbon nanotube material (CNT) in an amount ranging from 0.01 to 6.0 weight percent of the outer core. The inner mantle layer is disposed over the outer core. The inner mantle layer has a thickness ranging from 0.03 inch to 0.09 inch. The inner mantle layer material has a plaque Shore D hardness ranging from 36 to 44. The outer mantle layer is disposed over the inner mantle layer. The outer mantle layer has a thickness ranging from 0.025 inch to 0.070 inch. The outer mantle layer material has a plaque Shore D hardness ranging from 65 to 71. The inner mantle is thicker than the outer mantle, and the outer mantle is harder than the inner mantle. The cover layer is disposed over the outer mantle layer. The cover layer has a thickness ranging from 0.025 inch to 0.040 inch. The cover layer has a lower Shore D hardness than the outer mantle layer, the outer mantle layer has a higher Shore D hardness than the

inner mantle layer, and the outer core has a higher Shore D hardness than the inner mantle layer and the center core.

Yet another aspect of the present invention is a golf ball comprising a core, an inner mantle layer, a first center mantle layer, a second center mantle layer, an outer mantle layer, and a cover. The core comprises a polybutadiene material, a graphene material in an amount ranging from 0.01 to 6.0 weight percent of the core, and a carbon nanotube material (CNT) in an amount ranging from 0.01 to 6.0 weight percent of the core. The inner mantle layer is disposed over the core. The inner mantle layer has a thickness ranging from 0.030 inch to 0.050 inch. The inner mantle layer material has a plaque Shore D hardness ranging from 30 to 40. The inner mantle layer is composed of a composed of an ionomer material. The first center mantle layer is disposed over the inner mantle layer. The first center mantle layer has a thickness ranging from 0.030 inch to 0.050 inch. The first center mantle layer material has a plaque Shore D hardness ranging from 40 to 55. The first center mantle layer is composed of a fully neutralized polymer material. The second center mantle layer is disposed over the second center mantle layer. The second center mantle layer has a thickness ranging from 0.030 inch to 0.050 inch. The second center mantle layer material has a plaque Shore D hardness ranging from 45 to 55. The second center mantle layer is composed of a fully neutralized polymer material. The outer mantle layer is disposed over the second center mantle layer. The outer mantle layer has a thickness ranging from 0.030 inch to 0.050 inch. The outer mantle layer is composed of an ionomer material. The outer mantle layer material has a plaque Shore D hardness ranging from 60 to 75. The cover layer is disposed over the outer mantle layer, and has a thickness ranging from 0.025 inch to 0.040 inch.

A yet another aspect of the present invention is a method for forming a core for a golf ball. The method includes mixing a graphene material, a CNT material with a polybutadiene material to form a core mixture, wherein the graphene material ranges from 0.01 to 6.0 weight percent of the core mixture, and the CNT material ranges from 0.01 to 6.0 weight percent of the core mixture. The method also includes compression molding a core from the core mixture. The core preferably has a diameter ranging from 0.70 inch to 1.6 inch. The core mixture preferably comprises 40-90 weight percent of polybutadiene, 0.4 to 2.5 weight percent graphene material, 1-30 weight percent polyisoprene, 10-50 weight percent zinc diacrylate, 1-30 weight percent zinc oxide, 1-20 weight percent zinc stearate, and 0.1-10 weight percent peroxide initiator.

A more preferred embodiment of the method includes forming a cover over the core.

A more preferred embodiment of the method includes forming a mantle layer over the core.

A more preferred embodiment of the method includes that the core mixture is molded over an inner core to produce a dual core with a diameter ranging from 0.7 inch to 1.6 inches.

A more preferred embodiment of the method includes compression molding a core from the core mixture comprises compression molding an outer core layer over a center core comprising a polybutadiene mixture.

A more preferred embodiment of the method includes compression molding a core from the core mixture comprises compression molding a center core and an outer core over the center core, and the center core and the outer core comprise the core mixture.

Having briefly described the present invention, the above and further objects, features and advantages thereof will be

## 5

recognized by those skilled in the pertinent art from the following detailed description of the invention when taken in conjunction with the accompanying drawings.

BRIEF DESCRIPTION OF THE SEVERAL VIEWS OF THE DRAWINGS

FIG. 1 is an exploded partial cut-away view of a golf ball.  
FIG. 2 is top perspective view of a golf ball.

FIG. 3 is a cross-sectional view of a core component of a golf ball.

FIG. 4 is a cross-sectional view of a core component and a mantle component of a golf ball.

FIG. 5 is a cross-sectional view of an inner core layer, an outer core layer, an inner mantle layer, an outer mantle layer and a cover layer of a golf ball.

FIG. 5A is a cross-sectional view of an inner core layer, an intermediate core layer, an outer core layer, a mantle layer and a cover layer of a golf ball.

FIG. 6 is a cross-sectional view of an inner core layer under a 100 kilogram load.

FIG. 7 is a cross-sectional view of a core under a 100 kilogram load.

FIG. 8 is a cross-sectional view of a core component and a mantle component of a golf ball.

FIG. 9 is a cross-sectional view of a core component, the mantle component and a cover layer of a golf ball.

FIG. 10 is an exploded partial cut-away view of a four-piece golf ball.

FIG. 11 is an exploded partial cut-away view of a three-piece golf ball.

FIG. 12 is an exploded partial cut-away view of a two-piece golf ball.

FIG. 13 is a cross-sectional view of a two-piece golf ball.

FIG. 14 is a cross-sectional view of a three-piece golf ball.

FIG. 15 is an exploded partial cut-away view of a three-piece golf ball.

FIG. 16 is a cross-sectional view of a three-piece golf ball with a dual core and a cover.

FIG. 17 is a cross-sectional view of a three-piece golf ball with a core, mantle and cover.

FIG. 18 is a cross-sectional view of a four-piece golf ball with a dual core, mantle layer and a cover.

FIG. 19 is a cross-sectional view of a four-piece golf ball with a core, dual mantle layers and a cover.

FIG. 20 is a graph of durability testing of outer cores using PTM at 175 fps.

DETAILED DESCRIPTION OF THE INVENTION

The primary purpose of the present invention is to improve durability of golf ball core by incorporation of mixture of graphene and CNT in the core to improve the impact strength of the ball. This benefit can be seen in either a ball with single piece core, or a dual core with an outer core firmer than the inner core. Improved durability of the core by using a mixture of graphene and CNT can result in higher mean time to fail (MTTF) upon repeated impact in a high speed testing device, or with a golf club in normal play.

Another objective is to improve aging properties due to the incorporation of graphene in the core for better retention of compression and COR over time.

Polybutadiene based cores were made using following materials. Corresponding levels (by % wt) is mentioned next to each material: Polybutadiene with more than 60% 1,4-cis structure—(40-90%); Polyisoprene—(1-30%); Zinc diacyr-

## 6

late—(10-50%); Zinc oxide—(1-30%); Zinc stearate—(1-20%); Peroxide initiator—(0.1-10%); Zinc pentachlorothiophenol—(0-10%); Color—(0-10%); Barium sulfate—(0-20%); Graphene—(0.01-6%)—available from various suppliers such as Cheap Tubes Inc., Ad-Nano Technologies Private Limited, MKnano, XG Sciences Inc., Angstrom Materials Inc. which has a surface area between 150-1000 m<sup>2</sup>/g; Graphene masterbatch (a masterbatch with 5-95% polybutadiene or polyisoprene and 1-10% graphene)—(0.1-50%)—custom compounding can be done with the help of various suppliers such as Preferred Compounding Corp, Dyna-Mix, Alttran, Callaway (in house compounding; CNT—(0.01-6%)—available from various suppliers such as Bayer Material Science, Future Carbon, Cheap Tubes Inc, NanoAmor, Nanocyl, Nanocyl SA, Arkema, NanoTechLabs, Inc.; CNT masterbatch (a masterbatch of with 5-95% polyisoprene and 1-95% CNT)—(0.1-50%)—masterbatches or custom masterbatches are available from various suppliers such as Cheap Tubes Inc, Nanocyl SA, Arkema, NanoTechLabs, Inc.

Dual Cores with graphene/CNT in the outer core.

In this study graphene, CNT, and a mixture of graphene and CNT were introduced to the outer core in a dual core construction. Dual cores were made by compression molding two outer core halves around an already molded inner core having a diameter of approximately 0.940" and a soft compression of approximately 0.210 inches of deflection under a 200 lb load. Curing of the inner and outer core was done at temperatures ranging between 150-400 F for times ranging from 1-30 minutes. After molding, the dual cores were spherically ground to approximately 1.560" prior to testing.

Table 1 and 2 give details of recipe of inner and outer cores. Components from these recipes were mixed in an internal mixer. Optionally, additional mixing was done using a two roll mill.

Compression of the outer core is measured by first making a full size core separately, measuring its compression, and then molding two halves around the inner core to complete the dual core. Compression differential describes the difference between the outer core compression (as molded independently) and inner core compression. A higher compression differential is more susceptible to crack durability upon impact.

TABLE 1

| Inner core recipe          |       |  |
|----------------------------|-------|--|
| Components                 | % wt  |  |
| Polybutadiene rubber       | 70.1  |  |
| Polyisoprene rubber        | 0.0   |  |
| Zinc diacrylate            | 15.9  |  |
| Zinc oxide                 | 7.0   |  |
| 55 Zinc stearate           | 0.0   |  |
| Peroxide initiator         | 1.1   |  |
| Zinc pentachlorothiophenol | 0.6   |  |
| Color                      | 0.1   |  |
| Barium sulfate             | 0.0   |  |
| graphene                   | 0.0   |  |
| graphene masterbatch       | 0.0   |  |
| CNT                        | 0.0   |  |
| 60 CNT Masterbatch         | 0.0   |  |
| Properties                 |       |  |
| 65 Compression             | 0.210 |  |

TABLE 2

| Components                                                                                                 | Outer core recipe of dual core        |                                         |                                 |                                                          |
|------------------------------------------------------------------------------------------------------------|---------------------------------------|-----------------------------------------|---------------------------------|----------------------------------------------------------|
|                                                                                                            | Formula 1<br>(0%<br>Graphene)<br>% wt | Formula 2<br>(0.8%<br>Graphene)<br>% wt | Formula 3<br>(0.8% CNT)<br>% wt | Formula 4<br>(0.8%<br>Graphene + CNT<br>mixture)<br>% wt |
| Polybutadiene                                                                                              | 63.3                                  | 62.5                                    | 62.5                            | 62.5                                                     |
| Zinc Diacrylate                                                                                            | 26.3                                  | 26.9                                    | 26.9                            | 26.9                                                     |
| Zinc Oxide                                                                                                 | 6.3                                   | 5.9                                     | 5.9                             | 5.9                                                      |
| Zinc Stearate                                                                                              | 0.0                                   | 0.0                                     | 0.0                             | 0.0                                                      |
| Peroxide initiator                                                                                         | 0.5                                   | 0.5                                     | 0.5                             | 0.5                                                      |
| Zinc pentachlorothiophenol                                                                                 | 0.6                                   | 0.6                                     | 0.6                             | 0.6                                                      |
| Color                                                                                                      | 0.1                                   | 0.1                                     | 0.1                             | 0.1                                                      |
| Limestone                                                                                                  | 0.0                                   | 0.0                                     | 0.0                             | 0.0                                                      |
| Tungsten                                                                                                   | 0.0                                   | 0.0                                     | 0.0                             | 0.0                                                      |
| Barium sulfate                                                                                             | 2.9                                   | 2.8                                     | 2.8                             | 2.8                                                      |
| Graphene                                                                                                   | 0.0                                   | 0.0                                     | 0.0                             | 0.0                                                      |
| Graphene in masterbatch                                                                                    | 0.0                                   | 0.8                                     | 0.0                             | 0.4                                                      |
| CNT                                                                                                        | 0.0                                   | 0.0                                     | 0.0                             | 0.0                                                      |
| CNT added in masterbatch<br>form                                                                           | 0.0                                   | 0.0                                     | 0.8                             | 0.4                                                      |
| Properties of outer core                                                                                   |                                       |                                         |                                 |                                                          |
| Compression                                                                                                | 100.7                                 | 101.2                                   | 102.3                           | 102.2                                                    |
| COR (coefficient of<br>restitution)                                                                        | 0.816                                 | 0.809                                   | 0.806                           | 0.808                                                    |
| Properties of dual core built from inner and outer core                                                    |                                       |                                         |                                 |                                                          |
| Compression                                                                                                | 81.3                                  | 82.7                                    | 86.3                            | 85.1                                                     |
| COR (coefficient of restitution<br>@125 fps)                                                               | 0.812                                 | 0.808                                   | 0.808                           | 0.809                                                    |
| Durability score or mean time<br>to fail MTTF(number of shots<br>after which ball starts to<br>crack/fail) | 21                                    | 62                                      | 73                              | 65                                                       |

Compression is measured by applying a 200 pound load to the core and measuring its deflection, in inches. Compression=180-(deflection\*1000)

#### Durability Testing of Dual Cores

Cores were shot at 175 fps in a pneumatic testing machine (PTM).

For each formula mentioned in Table 2, 12 cores were tested. Number of shots after which each core cracked was recorded for each core, and the cracked core was removed from the remainder of the test. The data was reported using a Weibull plot, and the mean time to fail was reported as shown in Table 2. As seen in FIG. 1, graphene/CNT modified cores endured more shots before failure compared to cores with no graphene/CNT. It is reasonable to assume that the durability of a golf ball having a dual core of this design will also experience a dramatic increase in crack durability based on this improvement to the dual core. It is reasonable to assume that the addition of graphene/CNT in the inner core could provide a durability enhancement to the overall golf ball, but this study only focused on the outer core.

As our experiment has shown, incorporating graphene and CNT into the outer core recipe reinforces the strength of the outer core and provides greater crack durability protection in the design of a dual core golf ball, which is more susceptible to crack durability failures if the outer core is much firmer than the soft inner core.

FIGS. 1, 3, 4 and 5 illustrate a five piece golf ball 10 comprising an inner core 12a, an outer core 12b, an inner mantle 14a, an outer mantle 14b, and a cover 16, wherein the cover layer 16 is composed of a thermoplastic polyurethane. The intermediate core 12b comprises polybutadiene mixture comprising 0.4 to 2.5 weight percent of a graphene.

FIG. 5A illustrates a five piece golf ball 10 comprising an inner core 12a, an intermediate core 12b, an outer core 12c, a mantle 14, and a cover 16, wherein the cover layer 16 is composed of a thermoplastic polyurethane. The intermediate core 12b comprises polybutadiene mixture comprising 0.4 to 2.5 weight percent of a graphene.

FIGS. 8 and 9 illustrate a six piece golf ball 10 comprising an inner core 12a, an intermediate core 12b, an outer core 12c, an inner mantle 14a, an outer mantle 14b, and a cover 16, wherein the cover layer 16 is composed of a thermoplastic polyurethane. The inner core 12a comprises polybutadiene mixture comprising 0.4 to 2.5 weight percent of a graphene.

FIG. 10 illustrates a four piece golf ball comprising a dual core, a boundary layer and a cover. The outer core comprises polybutadiene mixture comprising 0.4 to 2.5 weight percent of a graphene.

FIG. 11 illustrates a three piece golf ball comprising a core, a boundary layer and a cover. The core comprises polybutadiene mixture comprising 0.4 to 2.5 weight percent of a graphene.

FIGS. 12 and 13 illustrate a two piece golf ball 20 with a core 25 and a cover 30. The core comprises polybutadiene mixture comprising 0.4 to 2.5 weight percent of a graphene.

FIGS. 14 and 15 illustrate a three-piece golf ball 5 comprising a core 10, a mantle layer 14 and a cover 16 with dimples 18, wherein the core comprises 0.4 to 2.5 weight percent of a graphene.

FIG. 16 illustrates a dual core three piece golf ball 35 comprising an inner core 30, and outer core 32 and a cover 34, wherein the core comprises 0.4 to 2.5 weight percent of a graphene.

FIG. 17 illustrates a three piece golf ball 45 comprising a core 40, a mantle layer 42 and a cover 44, wherein the core comprises 0.4 to 2.5 weight percent of a graphene.

FIG. 18 illustrates a dual core four piece golf ball 55 comprising an inner core 50, an outer core 52, a mantle layer 54 and a cover 56, wherein the core comprises 0.4 to 2.5 weight percent of a graphene.

FIG. 19 illustrates a four piece golf ball 65 comprising a core 60, an inner mantle 62, an outer mantle 64 and a cover 66, wherein the core comprises 0.4 to 2.5 weight percent of a graphene.

The mantle component is preferably composed of the inner mantle layer and the outer mantle layer. The mantle component preferably has a thickness ranging from 0.05 inch to 0.15 inch, and more preferably from 0.06 inch to 0.08 inch. The outer mantle layer is preferably composed of a blend of ionomer materials. One preferred embodiment comprises SURLYN 9150 material, SURLYN 8940 material, a SURLYN AD1022 material, and a masterbatch. The SURLYN 9150 material is preferably present in an amount ranging from 20 to 45 weight percent of the cover, and more preferably 30 to 40 weight percent. The SURLYN 8945 is preferably present in an amount ranging from 15 to 35 weight percent of the cover, more preferably 20 to 30 weight percent, and most preferably 26 weight percent. The SURLYN 9945 is preferably present in an amount ranging from 30 to 50 weight percent of the cover, more preferably 35 to 45 weight percent, and most preferably 41 weight percent. The SURLYN 8940 is preferably present in an amount ranging from 5 to 15 weight percent of the cover, more preferably 7 to 12 weight percent, and most preferably 10 weight percent.

SURLYN 8320, from DuPont, is a very-low modulus ethylene/methacrylic acid copolymer with partial neutralization of the acid groups with sodium ions. SURLYN 8945, also from DuPont, is a high acid ethylene/methacrylic acid copolymer with partial neutralization of the acid groups with sodium ions. SURLYN 9945, also from DuPont, is a high acid ethylene/methacrylic acid copolymer with partial neutralization of the acid groups with zinc ions. SURLYN 8940, also from DuPont, is an ethylene/methacrylic acid copolymer with partial neutralization of the acid groups with sodium ions.

The inner mantle layer is preferably composed of a blend of ionomers, preferably comprising a terpolymer and at least two high acid (greater than 18 weight percent) ionomers neutralized with sodium, zinc, magnesium, or other metal ions. The material for the inner mantle layer preferably has a Shore D plaque hardness ranging preferably from 35 to 77, more preferably from 36 to 44, a most preferably approximately 40. The thickness of the outer mantle layer preferably ranges from 0.025 inch to 0.050 inch, and is more preferably approximately 0.037 inch. The mass of an insert including the dual core and the inner mantle layer preferably ranges from 32 grams to 40 grams, more preferably from 34 to 38 grams, and is most preferably approximately 36 grams. The inner mantle layer is alternatively composed of a HPF material available from DuPont. Alternatively, the inner mantle layer 14b is composed of a material such as disclosed in Kennedy, III et al., U.S. Pat. No. 7,361,101 for a Golf Ball And Thermoplastic Material, which is hereby incorporated by reference in its entirety.

The outer mantle layer is preferably composed of a blend of ionomers, preferably comprising at least two high acid (greater than 18 weight percent) ionomers neutralized with sodium, zinc, or other metal ions. The blend of ionomers also preferably includes a masterbatch. The material of the

outer mantle layer preferably has a Shore D plaque hardness ranging preferably from 55 to 75, more preferably from 65 to 71, and most preferably approximately 67. The thickness of the outer mantle layer preferably ranges from 0.025 inch to 0.040 inch, and is more preferably approximately 0.030 inch. The mass of the entire insert including the core, the inner mantle layer and the outer mantle layer preferably ranges from 38 grams to 43 grams, more preferably from 39 to 41 grams, and is most preferably approximately 41 grams.

In an alternative embodiment, the inner mantle layer is preferably composed of a blend of ionomers, preferably comprising at least two high acid (greater than 18 weight percent) ionomers neutralized with sodium, zinc, or other metal ions. The blend of ionomers also preferably includes a masterbatch. In this embodiment, the material of the inner mantle layer has a Shore D plaque hardness ranging preferably from 55 to 75, more preferably from 65 to 71, and most preferably approximately 67. The thickness of the outer mantle layer preferably ranges from 0.025 inch to 0.040 inch, and is more preferably approximately 0.030 inch. Also in this embodiment, the outer mantle layer 14b is composed of a blend of ionomers, preferably comprising a terpolymer and at least two high acid (greater than 18 weight percent) ionomers neutralized with sodium, zinc, magnesium, or other metal ions. In this embodiment, the material for the outer mantle layer 14b preferably has a Shore D plaque hardness ranging preferably from 35 to 77, more preferably from 36 to 44, a most preferably approximately 40. The thickness of the outer mantle layer preferably ranges from 0.025 inch to 0.100 inch, and more preferably ranges from 0.070 inch to 0.090 inch.

In yet another embodiment wherein the inner mantle layer is thicker than the outer mantle layer and the outer mantle layer is harder than the inner mantle layer, the inner mantle layer is composed of a blend of ionomers, preferably comprising a terpolymer and at least two high acid (greater than 18 weight percent) ionomers neutralized with sodium, zinc, magnesium, or other metal ions. In this embodiment, the material for the inner mantle layer has a Shore D plaque hardness ranging preferably from 30 to 77, more preferably from 30 to 50, and most preferably approximately 40. In this embodiment, the material for the outer mantle layer has a Shore D plaque hardness ranging preferably from 40 to 77, more preferably from 50 to 71, and most preferably approximately 67. In this embodiment, the thickness of the inner mantle layer preferably ranges from 0.030 inch to 0.090 inch, and the thickness of the outer mantle layer ranges from 0.025 inch to 0.070 inch.

Preferably the inner core has a diameter ranging from 0.75 inch to 1.20 inches, more preferably from 0.85 inch to 1.05 inch, and most preferably approximately 0.95 inch. Preferably the inner core 12a has a Shore D hardness ranging from 20 to 50, more preferably from 25 to 40, and most preferably approximately 35. Preferably the inner core has a mass ranging from 5 grams to 15 grams, 7 grams to 10 grams and most preferably approximately 8 grams.

Preferably the outer core has a diameter ranging from 1.25 inch to 1.55 inches, more preferably from 1.40 inch to 1.5 inch, and most preferably approximately 1.5 inch. Preferably the outer core has a Shore D surface hardness ranging from 40 to 65, more preferably from 50 to 60, and most preferably approximately 56. Preferably the outer core is formed from a polybutadiene, zinc diacrylate, zinc oxide, zinc stearate, a peptizer and peroxide. Preferably the combined inner core and outer core have a mass ranging from 25 grams to 35 grams, 30 grams to 34 grams and most preferably approximately 32 grams.

## 11

Preferably the inner core has a deflection of at least 0.230 inch under a load of 220 pounds, and the core has a deflection of at least 0.080 inch under a load of 200 pounds. As shown in FIGS. 6 and 7, a mass 50 is loaded onto an inner core and a core. As shown in FIGS. 6 and 7, the mass is 100 kilograms, approximately 220 pounds. Under a load of 100 kilograms, the inner core preferably has a deflection from 0.230 inch to 0.300 inch. Under a load of 100 kilograms, preferably the core has a deflection of 0.08 inch to 0.150 inch. Alternatively, the load is 200 pounds (approximately 90 kilograms), and the deflection of the core 12 is at least 0.080 inch. Further, a compressive deformation from a beginning load of 10 kilograms to an ending load of 130 kilograms for the inner core ranges from 4 millimeters to 7 millimeters and more preferably from 5 millimeters to 6.5 millimeters. The dual core deflection differential allows for low spin off the tee to provide greater distance, and high spin on approach shots.

In an alternative embodiment of the golf ball shown in FIG. 5A, the golf ball 10 comprises an inner core 12a, an intermediate core 12b, an outer core 12b, a mantle 14 and a cover 16. The golf ball 10 preferably has a diameter of at least 1.68 inches, a mass ranging from 45 grams to 47 grams, a COR of at least 0.79, a deformation under a 100 kilogram loading of at least 0.07 mm.

In one embodiment, the golf ball comprises a core, a mantle layer and a cover layer. The core comprises an inner core sphere, an intermediate core layer and an outer core layer. The intermediate core layer is composed of a highly neutralized ionomer and has a Shore D hardness less than 40. The outer core layer is composed of a highly neutralized ionomer and has a Shore D hardness less than 45. A thickness of the intermediate core layer is greater than a thickness of the outer core layer. The mantle layer is disposed over the core, comprises an ionomer material and has a Shore D hardness greater than 55. The cover layer is disposed over the mantle layer comprises a thermoplastic polyurethane material and has a Shore A hardness less than 100. The golf ball has a diameter of at least 1.68 inches. The mantle layer is harder than the outer core layer, the outer core layer is harder than the intermediate core layer, the intermediate core layer is harder than the inner core sphere, and the cover layer is softer than the mantle layer.

In another embodiment, shown in FIGS. 8 and 9, the golf ball 10 has a multi-layer core and multi-layer mantle. The golf ball includes a core, a mantle component and a cover layer. The core comprises an inner core sphere, an intermediate core layer and an outer core layer. The inner core sphere comprises a TPEE material and has a diameter ranging from 0.875 inch to 1.4 inches. The intermediate core layer is composed of a highly neutralized ionomer and has a Shore D hardness less than 40. The outer core layer is composed of a highly neutralized ionomer and has a Shore D hardness less than 45. A thickness of the intermediate core layer is greater than a thickness of the outer core layer 12c. The inner mantle layer is disposed over the core, comprises an ionomer material and has a Shore D hardness greater than 55. The outer mantle layer is disposed over the inner mantle layer, comprises an ionomer material and has a Shore D hardness greater than 60. The cover layer is disposed over the mantle component, comprises a thermoplastic polyurethane material and has a Shore A hardness less than 100. The golf ball has a diameter of at least 1.68 inches. The outer mantle layer is harder than the inner mantle layer, the inner mantle layer is harder than the outer core layer, the outer core layer is harder than the intermediate core layer, the

## 12

intermediate core layer is harder than the inner core sphere, and the cover layer is softer than the outer mantle layer.

In a particularly preferred embodiment of the invention, the golf ball preferably has an aerodynamic pattern such as disclosed in Simonds et al., U.S. Pat. No. 7,419,443 for a Low Volume Cover For A Golf Ball, which is hereby incorporated by reference in its entirety. Alternatively, the golf ball has an aerodynamic pattern such as disclosed in Simonds et al., U.S. Pat. No. 7,338,392 for An Aerodynamic Surface Geometry For A Golf Ball, which is hereby incorporated by reference in its entirety.

Various aspects of the present invention golf balls have been described in terms of certain tests or measuring procedures. These are described in greater detail as follows.

As used herein, "Shore D hardness" of the golf ball layers is measured generally in accordance with ASTM D-2240 type D, except the measurements may be made on the curved surface of a component of the golf ball, rather than on a plaque. If measured on the ball, the measurement will indicate that the measurement was made on the ball. In referring to a hardness of a material of a layer of the golf ball, the measurement will be made on a plaque in accordance with ASTM D-2240. Furthermore, the Shore D hardness of the cover is measured while the cover remains over the mantles and cores. When a hardness measurement is made on the golf ball, the Shore D hardness is preferably measured at a land area of the cover.

As used herein, "Shore A hardness" of a cover is measured generally in accordance with ASTM D-2240 type A, except the measurements may be made on the curved surface of a component of the golf ball, rather than on a plaque. If measured on the ball, the measurement will indicate that the measurement was made on the ball. In referring to a hardness of a material of a layer of the golf ball, the measurement will be made on a plaque in accordance with ASTM D-2240. Furthermore, the Shore A hardness of the cover is measured while the cover remains over the mantles and cores. When a hardness measurement is made on the golf ball, Shore A hardness is preferably measured at a land area of the cover.

The resilience or coefficient of restitution (COR) of a golf ball is the constant "e," which is the ratio of the relative velocity of an elastic sphere after direct impact to that before impact. As a result, the COR ("e") can vary from 0 to 1, with 1 being equivalent to a perfectly or completely elastic collision and 0 being equivalent to a perfectly or completely inelastic collision.

COR, along with additional factors such as club head speed, club head mass, ball weight, ball size and density, spin rate, angle of trajectory and surface configuration as well as environmental conditions (e.g. temperature, moisture, atmospheric pressure, wind, etc.) generally determine the distance a ball will travel when hit. Along this line, the distance a golf ball will travel under controlled environmental conditions is a function of the speed and mass of the club and size, density and resilience (COR) of the ball and other factors. The initial velocity of the club, the mass of the club and the angle of the ball's departure are essentially provided by the golfer upon striking. Since club head speed, club head mass, the angle of trajectory and environmental conditions are not determinants controllable by golf ball producers and the ball size and weight are set by the U.S.G.A., these are not factors of concern among golf ball manufacturers. The factors or determinants of interest with respect to improved distance are generally the COR and the surface configuration of the ball.

The coefficient of restitution is the ratio of the outgoing velocity to the incoming velocity. In the examples of this application, the coefficient of restitution of a golf ball was measured by propelling a ball horizontally at a speed of 125+/-5 feet per second (fps) and corrected to 125 fps against a generally vertical, hard, flat steel plate and measuring the ball's incoming and outgoing velocity electronically. Speeds were measured with a pair of ballistic screens, which provide a timing pulse when an object passes through them. The screens were separated by 36 inches and are located 25.25 inches and 61.25 inches from the rebound wall. The ball speed was measured by timing the pulses from screen 1 to screen 2 on the way into the rebound wall (as the average speed of the ball over 36 inches), and then the exit speed was timed from screen 2 to screen 1 over the same distance. The rebound wall was tilted 2 degrees from a vertical plane to allow the ball to rebound slightly downward in order to miss the edge of the cannon that fired it. The rebound wall is solid steel.

As indicated above, the incoming speed should be 125±5 fps but corrected to 125 fps. The correlation between COR and forward or incoming speed has been studied and a correction has been made over the ±5 fps range so that the COR is reported as if the ball had an incoming speed of exactly 125.0 fps.

The measurements for deflection, compression, hardness, and the like are preferably performed on a finished golf ball as opposed to performing the measurement on each layer during manufacturing.

Preferably, in a five layer golf ball comprising an inner core, an outer core, an inner mantle layer, an outer mantle layer and a cover, the hardness/compression of layers involve an inner core with the greatest deflection (lowest hardness), an outer core (combined with the inner core) with a deflection less than the inner core, an inner mantle layer with a hardness less than the hardness of the combined outer core and inner core, an outer mantle layer with the hardness layer of the golf ball, and a cover with a hardness less than the hardness of the outer mantle layer. These measurements are preferably made on a finished golf ball that has been torn down for the measurements.

Preferably the inner mantle layer is thicker than the outer mantle layer or the cover layer. The dual core and dual mantle golf ball creates an optimized velocity-initial velocity ratio (Vi/IV), and allows for spin manipulation. The dual core provides for increased core compression differential resulting in a high spin for short game shots and a low spin for driver shots. A discussion of the USGA initial velocity test is disclosed in Yagley et al., U.S. Pat. No. 6,595,872 for a Golf Ball With High Coefficient Of Restitution, which is hereby incorporated by reference in its entirety. Another example is Bartels et al., U.S. Pat. No. 6,648,775 for a Golf Ball With High Coefficient Of Restitution, which is hereby incorporated by reference in its entirety.

From the foregoing it is believed that those skilled in the pertinent art will recognize the meritorious advancement of this invention and will readily understand that while the present invention has been described in association with a preferred embodiment thereof, and other embodiments illustrated in the accompanying drawings, numerous changes, modifications and substitutions of equivalents may be made therein without departing from the spirit and scope of this invention which is intended to be unlimited by the foregoing except as may appear in the following appended claims. Therefore, the embodiments of the invention in which an exclusive property or privilege is claimed are defined in the following appended claims.

We claim as our invention the following:

1. A golf ball comprising:  
an inner core comprising a polybutadiene material;  
an outer core comprising a polybutadiene in an amount ranging from 40 to 90 weight percent, zinc diacrylate in an amount ranging from 10 to 50 weight percent, zinc oxide in an amount ranging from 1 to 30 weight percent, peroxide initiator in an amount ranging from 0.1 to 10 weight percent, a graphene material in an amount ranging from 0.01 to 6.0 weight percent of the outer core, and a carbon nanotube (CNT) material in an amount ranging from 0.01 to 6.0 weight percent of the outer core, wherein the graphene material has a surface area ranging from 150 m<sup>2</sup>/g to 1000 m<sup>2</sup>/g; and a cover layer disposed over the outer core.

2. The golf ball according to claim 1 wherein the graphene material ranges from 0.4 to 1.0 weight percent of the outer core.

3. The golf ball according to claim 1 wherein the graphene material ranges from 0.4 to 0.8 weight percent of the outer core.

4. The golf ball according to claim 1 wherein the CNT material ranges from 0.4 to 0.8 weight percent of the outer core.

5. The golf ball according to claim 1 wherein the CNT material ranges from 0.4 to 1.0 weight percent of the outer core.

6. The golf ball according to claim 1 further comprising: an inner mantle layer disposed over the outer core, the inner mantle layer having a thickness ranging from 0.03 inch to 0.09 inch, the inner mantle layer composed of an ionomer material, the inner mantle layer material having a plaque Shore D hardness ranging from 34 to 55;

an outer mantle layer disposed over the inner mantle layer, the outer mantle layer having a thickness ranging from 0.025 inch to 0.050 inch; and

wherein the cover layer is disposed over the outer mantle layer, the cover layer has a thickness ranging from 0.025 inch to 0.040 inch;

wherein the cover layer has a lower Shore D hardness than the outer mantle layer, the outer mantle layer has a higher Shore D hardness than the inner mantle layer, the outer core has a higher Shore D hardness than the inner mantle layer and the inner core.

7. The golf ball according to claim 1 further comprising: an inner mantle layer disposed over the outer core, the inner mantle layer having a thickness ranging from 0.030 inch to 0.090 inch, the inner mantle layer material having a plaque Shore D hardness ranging from 30 to 50;

an outer mantle layer disposed over the inner mantle layer, the outer mantle layer having a thickness ranging from 0.025 inch to 0.070 inch, the outer mantle layer material having a plaque Shore D hardness ranging from 50 to 71, wherein the inner mantle is thicker than the outer mantle, and the outer mantle is harder than the inner mantle; and

wherein the cover layer is disposed over the outer mantle layer, the cover layer having a thickness ranging from 0.025 inch to 0.050 inch, wherein the cover layer has a Shore D hardness less than the hardness of the outer mantle layer, the outer mantle layer has a higher Shore D hardness than the inner mantle layer, the outer core has a higher Shore D hardness than the inner mantle layer and the center core.

**15**

8. The golf ball according to claim 1 further comprising: an inner mantle layer disposed over the outer core, the inner mantle layer having a thickness ranging from 0.070 inch to 0.090 inch, the inner mantle layer composed of an ionomer material, the inner mantle layer material having a plaque Shore D hardness ranging from 36 to 44; 5  
an outer mantle layer disposed over the inner mantle layer, the outer mantle layer having a thickness ranging from 0.025 inch to 0.040 inch, the outer mantle layer composed of an ionomer material, the outer mantle layer material having a plaque Shore D hardness ranging from 65 to 71; and  
wherein the cover layer is disposed over the outer mantle layer, the cover layer having a thickness ranging from 0.025 inch to 0.040 inch; 15  
wherein the cover layer has a lower Shore D hardness than the outer mantle layer, the outer mantle layer has a higher Shore D hardness than the inner mantle layer, the outer core has a higher Shore D hardness than the inner mantle layer and the center core.
9. The golf ball according to claim 1 wherein a core comprising the inner core and the outer core has a compression value ranging from 40 to 55.

10. The golf ball according to claim 1 further comprising: 25  
an inner mantle layer disposed over the center core, the inner mantle layer having a thickness ranging from 0.030 inch to 0.050 inch, the inner mantle layer material having a plaque Shore D hardness ranging from 30 to 40, the inner mantle layer composed of an ionomer material;  
a first center mantle layer disposed over the inner mantle layer, the first center mantle layer having a thickness ranging from 0.030 inch to 0.050 inch, the first center mantle layer material having a plaque Shore D hardness ranging from 40 to 55, the first center mantle layer composed of a fully neutralized polymer material; 30  
a second center mantle layer disposed over the second center mantle layer, the second center mantle layer having a thickness ranging from 0.030 inch to 0.050 inch;

**16**

- inch, the second center mantle layer material having a plaque Shore D hardness ranging from 45 to 55, the second center mantle layer composed of a fully neutralized polymer material; 5  
an outer mantle layer disposed over the second center mantle layer, the outer mantle layer having a thickness ranging from 0.030 inch to 0.050 inch, the outer mantle layer composed of a blend of ionomers, the outer mantle layer material having a plaque Shore D hardness ranging from 60 to 75; and  
wherein the cover layer is disposed over the outer mantle layer, the cover layer having a thickness ranging from 0.025 inch to 0.040 inch.
11. A golf ball comprising:  
an inner core comprising a polybutadiene material;  
an outer core comprising a polybutadiene in an amount ranging from 40 to 90 weight percent, zinc diacrylate in an amount ranging from 10 to 50 weight percent, zinc oxide in an amount ranging from 1 to 30 weight percent, peroxide initiator in an amount ranging from 0.1 to 10 weight percent, a graphene material in an amount ranging from 0.01 to 6.0 weight percent of the outer core, and a carbon nanotube (CNT) material in an amount ranging from 0.01 to 6.0 weight percent of the outer core, wherein the graphene material has a surface area ranging from 150 m<sup>2</sup>/g to 1000 m<sup>2</sup>/g;  
a mantle layer; and  
a cover.
12. The golf ball according to claim 11 wherein the mantle layer comprises an inner mantle layer and an outer mantle layer.
13. The golf ball according to claim 11 wherein the graphene material in the outer core ranges from 0.4 to 0.8 weight percent of the outer core, and wherein the CNT material in the outer core ranges from 0.4 to 0.8 weight percent of the inner core.
14. The golf ball according to claim 11 wherein a core comprising the inner core and the outer core has a compression value ranging from 40 to 55.

\* \* \* \* \*